

# UNITED STATES PATENT OFFICE.

MILTON F. LINDSLEY, OF NORTH BERGEN, NEW JERSEY.

## PROCESS OF MAKING EXPLOSIVE COMPOUNDS.

SPECIFICATION forming part of Letters Patent No 341,155, dated May 4, 1886

Application filed November 30, 1885. Serial No. 184,346. (No specimens.)

To all whom it may concern:

Be it known that I, MILTON FLETCHER LINDSLEY, of North Bergen, (West Hoboken P. O.) in the county of Hudson and State 5 of New Jersey, have invented a new and Improved Process for Making Explosive Compounds, of which the following is a full, clear, and exact description.

The object of this invention is to provide 10 explosive compounds that can be used in all kinds of fire-arms, that will not develop any abnormal pressure upon the walls of the arms, and that will not foul the arms or produce any corrosive effect thereon.

15 The invention consists in first forming a mechanical mixture of wood fiber, charcoal, bituminous coal, and starch, grinding the mixture into powder, forming the powder into grains, treating the grains with acids, neutralizing them, drying them, and treating them in 20 a solution of carbonate of potash and saltpeter, as will be hereinafter fully described.

In applying my invention to practical use, I reduce wood fiber to a pulp by any of the 25 well-known means that do not require chemicals in their application, and boil the pulp in a twenty per cent. (20%) solution of carbonate of soda, to remove all foreign and resinous substances, and then thoroughly wash it in 30 pure cold water by the use of a filter-press, and then dry it by any suitable means.

The wood fiber, charcoal, bituminous coal, and starch are placed in an iron cylinder, or 35 other suitable receptacle, to be reduced to a fine powder. The iron cylinder is mounted on trunnions, and is connected by suitable gearing with a counter-shaft, by which it is driven at about the rate of twenty revolutions per minute.

40 In making up the charge for the cylinder, I use the ingredients in about the following quantities and proportions, viz: wood fiber, seventy-one pounds; charcoal, fourteen pounds, bituminous coal, five pounds; starch, ten 45 pounds.

I do not limit myself to the exact proportions given, as the density of the powder can be increased by increasing the proportional quantity of the bituminous coal; or the quantity of bituminous coal can be lessened and

its place supplied with glucose when a powder of less density is required.

The iron cylinder is provided upon its inner surface with iron projections, and about eight hundred pounds of iron balls are put 55 into it with the charge, so that the charge will be reduced to a fine powder by the action of the said balls and projections as the said cylinder is revolved upon its axis, and at the same time the several ingredients will be thoroughly 60 mixed. This operation should be continued for about ten hours.

To the fine powder thus produced I add enough water to form a mixture, when thoroughly mixed, of about the consistency of 65 dough. This mass is then formed into grains or granules by means of the apparatus herein-after described, or by any other suitable means.

A box, about five feet long and two feet wide, is mounted on legs fitted into iron  $\text{V}$ -shaped grooves in which they slide. The box is covered by a steel-wire sieve having ten meshes to the inch. The bottom of the box is made at an inclination of about twenty degrees (20°), and to the end of the box is secured an 70 apron having an inclination of about twenty degrees, (20°,) and forming a continuation of the box-bottom. The end of the box under the sieve and next the apron is left open, and upon the sieve is placed a second box, fitted 75 within the sieve-frame. To the opposite end of the box from the apron is secured the end of a connecting-rod, the other end of which is pivoted to a crank on the counter-shaft, by which it is driven, so that the apparatus will 80 receive a reciprocating movement from the shaft, which should make about one hundred and twenty revolutions per minute. About ten pounds of the dough-like mixture is put 85 into the sieve at a time, and also a number of iron balls, so that the mixture will be forced by the action of the balls through the sieve in small particles, which fall upon the inclined bottom of the box, roll off upon the inclined apron, and fall thence into a receptacle placed 90 beneath the said apron to receive them. The grains thus formed are thoroughly dried, and are then ready for the acid bath, which is formed of two hundred pounds of nitric acid 95 of fifty degrees (50°) Baumé, and four hundred 100

pounds of sulphuric acid of sixty-six and a half degrees ( $66\frac{1}{2}^{\circ}$ ) Baumé for each one hundred pounds of the grains, and into which the grains are slowly mixed, and where they are allowed to steep a sufficient length of time to permit a chemical change of all the ingredients except the charcoal, which generally requires about four hours. The grains are then washed in clean water till as much as possible of the free acid is removed, and are then subjected to a number of hot-water and alkaline baths, to more thoroughly remove the free acid.

When the free acid is completely removed or neutralized, the grains are taken to a dry-  
15 ing-room, where they are kept at a tempera-  
ture of about one hundred and twenty degrees  
( $120^{\circ}$ ) Fahrenheit, until thoroughly dried.  
The dried grains are then treated in a solution  
20 of carbonate of potash and saltpeter, or chlo-  
rate of potash, or both, and are again dried,  
and are then ready for use.

The wood fiber is generally prepared in the  
form of pulp from some light fibrous wood,  
preferably poplar, by any of the well-known  
25 processes for this purpose. The process used  
for making paper-stock will generally answer  
the purpose, but care must be taken that no  
chemicals be used in its preparation.

The charcoal is prepared from some light  
30 fibrous wood, preferably willow, in an iron  
retort, care being taken not to allow the tem-  
perature to rise above eight hundred degrees  
( $800^{\circ}$ ) Fahrenheit.

The bituminous coal used is the kind gen-  
35 erally employed for making steam, care being  
taken to have it free from slate and other  
foreign substances.

The starch preferably used is prepared from  
corn.

40 The glucose, when used, should preferably  
be prepared from corn.

By this process an explosive compound is  
prepared, in which the main explosive agent  
is nitrocellulose, but which is perfectly safe to  
45 use in fire-arms. This is accomplished by  
having each atom of the nitro-cellulose sur-

rounded by or in contact with an atom of car-  
bon, which retards or checks the gases of the  
nitro-cellulose, and at the same time helps to  
keep up the temperature of the explosion or 50  
combustion.

The bituminous coal is used to add to the  
density of the powder, and at the same time  
to furnish available gases to add to the bal-  
listic or driving force of the explosion. The 55  
glucose, when used, is for the same purpose.  
The starch, being a glutinous substance, binds  
the particles together and makes the grains  
harder and more dense and not so liable to  
crumble to dust, and which when the grains 60  
are treated with the acids forms a nitro com-  
pound which adds to the force of the explo-  
sion.

The carbonate of potash is used for the pur-  
pose of keeping the compound neutral, and 65  
thereby preventing decomposition.

The saltpeter is used to furnish oxygen for  
the complete combustion of the nitro-cellulose  
and at the same time to form with the carbon  
a second explosive body.

The powder prepared by this process is  
perfectly safe to use in fire-arms of all kinds,  
and will not develop any abnormal pressure  
on the walls of the fire-arms in which it is  
used, and will not foul the arms or produce 75  
any corrosive action thereon.

Having thus described my invention, I claim  
as new and desire to secure by Letters Patent—

The process for making explosive com-  
pounds herein described, which consists in 80  
forming a mechanical mixture of wood fiber,  
charcoal, bituminous coal, and starch, then  
forming the mixture into a fine powder, then  
treating the grains with acids, then removing 85  
the free acid, and then treating the grains in a  
solution of carbonate of potash and saltpeter,  
substantially as set forth.

MILTON F. LINDSLEY.

Witnesses:

JAMES T. GRAHAM,  
C. SEDGWICK.